

## UNITED STATES PATENT OFFICE

2,367,360

PROCESS OF CURING BRIER FOR PIPE  
MANUFACTURE

David P. Lavietes, Brooklyn, N. Y.

No Drawing. Application February 3, 1942,  
Serial No. 429,398

1 Claim. (Cl. 117—59)

The invention relates to a process of curing brier for pipe manufacture, and more particularly to a treatment of blocks cut from the burls of rhododendron, kalmia and similar brier woods.

For some years past, brierwood found in North Africa has not been readily available in this country because of the difficulties of importation. This imported brierwood, because of climatic and other conditions at its point of origin, is particularly adapted for use in the manufacture of pipes, since it is thoroughly cured by nature and is highly resistant to charring when in use as a pipe bowl.

American-grown brier, such as rhododendron, kalmia, etc. has been found not to give satisfactory results since the conditions of its growth are not such as to so cure or season the wood as to prevent its rapid charring or burning while a pipe is in use, and because of its tendency to warp and crack when subjected to heat.

In the production of pipe bowls made of brier blocks, the wood cut from the burls has to be turned, frazed and bored to give it the desired shape before final polishing and finishing, and wastage is high if defects in the block are not discovered until during the turning and frazing operations.

I have found that the blocks produced from rhododendron, kalmia, etc. burls, contain acids, and possibly resins, preventing a proper curing or seasoning of the brierwood, and a proper treatment making this wood highly resistant to the heat and fire to which it is subjected while a pipe is in use.

By actual production of the brier blocks for the manufacture of pipes in large quantities, I have found that such wood may be so conditioned in a short time as compared with that required for the natural conditioning of the wood, which time is of unknown duration, and that wood so conditioned will approximate the qualities of the naturally cured wood so far as the procedure followed in producing pipes from such wood and the durability of pipes made therefrom, are concerned.

The native brier has a grain and takes a finish, quite as attractive as the imported brier. In fact, a pipe produced from native brier, when cured and seasoned by the process of my invention, is at least equal in appearance and durability, to pipes made from imported brier.

The process of my invention is such as to not only remove the natural acids and possibly resins from the brier, but to prevent warping and cracking thereof during and following the treat-

ment, and ensure a thorough impregnation of the blocks with the chemical agent used for imparting fire retardant properties to the wood.

The invention consists primarily in a process of curing brier for pipe manufacture consisting in subjecting a block cut from the rhododendron, kalmia or other brier burl, to an aqueous solvent for acids, resins or other soluble constituents of the wood at an elevated temperature to remove such constituents therefrom, transferring said blocks while still saturated with said solvent, to aqueous solution containing a fire retardant agent soluble by said aqueous solvent maintained at an elevated temperature, and finally slowly drying said blocks; and in such other further steps and practices as are hereinafter set forth and described, and more particularly pointed out in the claims hereto appended.

In the process of the invention, brier blocks of a size to produce the stummels are cured or seasoned prior to the turning, frazing and boring operations incidental to the production of the stummels. This process is an artificial aging method which results in the production, in a few weeks, of a product equal, if not superior, to the natural imported brierwood.

To accomplish this result, it is essential to remove from substantially all of the wood of the block, the acids and other soluble constituents, including possibly resins, and to impregnate substantially the entire wood of the block with a fire retardant agent. I refer to substantially the entire wood of the block, although it is quite unimportant whether the conditions at the core of the block are the same as more toward the surface thereof, since in boring, this core portion is removed.

The blocks are rough hewn, according to the shape of stummel desired, thus ensuring the desired conditioning of the portion of the block constituting the stummel, particularly about the upper portion of the bowl of a pipe.

Blocks formed as above are first placed in a barrel or tank open to atmosphere, and subjected to a liquid solvent for the acids or other ingredients to be removed from the wood. I have found, in actual practice, that ordinary reservoir water, maintained at the temperature of substantially its boiling point, is highly effective. This treatment continues for a period of from six to ten hours, the water being brought to the boiling point after the immersion of the blocks therein, and the temperature thereof, after the water has once boiled, being maintained by the injection of live steam thereinto. Gurgita-

tion minimizes settling of sediment upon the surface of the blocks, although this is not a matter of major importance.

Experience has shown that with the time intervals stated, the block will become saturated throughout with the water or other solvent, and a high percentage of the deleterious ingredients in the wood will be removed.

After this step in the process, the blocks, before there has been an opportunity for any substantial evaporation of the solvent therefrom, particularly that portion of the solvent toward the center of the block, are subjected to a bath containing in solution a fireproofing agent, specifically boric acid. The quantity of boric acid in the solution will vary according to the character of the wood being treated.

The wood of blocks cut from the rhododendron burl, being soft and coarse grained as compared with the wood of blocks cut from kalmia burls, not only require shorter time intervals in the treatment, but a lower boric acid content in the bath. With kalmia, I have found that a boric acid content of approximately 25% gives the best results, but with the rhododendron wood this content may be much lower. I have also found that the immediate transfer of the solvent saturated blocks from the treatment barrel or tank to the boric acid bath is preferable, although a delay of forty-eight hours or so is not prohibitive.

While the blocks are in the boric acid bath, this bath is maintained at the temperature of the boiling point of water. I have heretofore maintained this temperature by means of steam coils in the barrels or tanks, since this prevents dilution of the fire retardant solution.

Again, according to the character of the wood in the blocks, the time intervals of this treatment may vary from approximately fourteen to twenty hours, this ordinarily being sufficient to ensure the impregnation of substantially the entire block with the boric acid solution. This is assisted by the water with which the block is saturated, and carries the degree of penetration or impregnation of the boric acid solution to the very center of the block.

By a rough pre-shaping of the blocks as stated, the penetration of the boric acid solution to all portions of the block used in forming the bowl of a pipe, in sufficient quantity to secure the desired fire resistant properties of this portion of the bowl, is assured. It has been found in actual practice that when a pipe bowl has been bored, the presence of the boric acid in the inner wall thereof is clearly visible, even to the naked eye, before the final finishing of the bowl.

After the blocks have been subjected to the boric acid bath for the necessary period, they are removed from the bath and allowed to dry slowly at a slightly elevated temperature, or in a warm room, to complete the curing or seasoning operation. I have found that this drying out operation should continue for some eight weeks or more to permit the turning, fazing and boring operations without likelihood of the subsequent warping and cracking of the wood of a pipe bowl. This is probably due to the fact that with a long curing or seasoning operation, substantially all moisture is evaporated from the wood, leaving only the precipitate of the boric acid in the pores of the wood.

The time intervals herein given are merely approximate, since the operation can be accelerated by the use of pressure tanks instead of using barrels or tanks open to atmosphere, or by

well known practices for accelerating evaporation.

The time intervals stated are those which I have actually used in producing treated blocks, and with a plant in continuing operation, time intervals are not factors of major importance.

I have found the use of heated baths to be essential in the first two steps of the process, but believe that the exact temperatures of these baths 10 is not critical so long as they are approximately the boiling point of water. The temperatures stated are those used with barrels or tanks open to atmosphere. It would be possible, however, to use a lower temperature if subatmospheric pressure were maintained in the barrels or tanks.

While I have found, in actual practice, that a 25% solution of boric acid gives the best results with harder and closer grained briars, this percentage may be lowered when treating the wood 20 of rhododendron burls. I believe that under some conditions, as low as a 10% solution of boric acid may be effectively used by increasing the time intervals.

In the practice of the process, the solution used 25 should be closely checked at intervals of approximately two hours, and fresh boric acid added if necessary. The solution may be repeatedly used.

It has been found that longer time intervals 30 are required to properly condition blocks of larger dimensions than smaller blocks.

In preparing the blocks, the burls are first carefully inspected to remove stones and dirt, and then sawed into slabs of a thickness approximating the height of block required for stummels of the desired sizes. These slabs are then cut into strips of a width required in the production of stummels of the size permissible with the thickness of the slab.

Skilled workmen then cut these strips into the greatest possible length, in view of imperfections in the strips.

In this way, a large variety of blocks of different sizes for the production of stummels of different forms, is obtained. The larger blocks 45 command relatively much greater prices than smaller blocks.

When treating blocks, they are selected according to size, and the time intervals vary accordingly.

It is not my intention to limit the invention to the precise time intervals herein stated, nor to the exact boric acid content, except approximately within the range stated. I have found 55 it essential, however, to subject the blocks to a bath at an elevated temperature to remove acids and other ingredients therefrom and saturate the blocks with water or other solvent; to place the blocks in a boric acid bath maintained at an elevated temperature before the water or other solvent has had an opportunity to evaporate, and finally to remove the vehicle for the boric acid by slow drying.

The specific temperatures, percentages and 60 time intervals herein stated may be varied according to the characteristics of the brierwood being treated, and the size of the blocks, so that it is not my intention to limit the invention to such specific details.

Having described the invention, what I claim as new and desire to have protected by Letters Patent is:

A process of curing brier for pipe manufacture consisting in subjecting a block cut from the 75 rhododendron, kalmia or other brier burl, for

from six to ten hours to water maintained substantially at its boiling point to remove acids, resins or other soluble constituents therefrom, maintaining the temperature of said water by a continuing delivery of live steam thereinto, transferring said blocks while still saturated with water to an aqueous solution containing boric acid within a range of from 10% to 25% of the volume of the bath, at an elevated temperature for a time interval within the range of fourteen to

20 twenty hours, maintaining said solution at substantially the boiling point of water and at a substantially uniform density by subjecting same to a dry heat, and finally drying said blocks for a time interval of approximately eight weeks at a low temperature to evaporate the liquid therefrom and precipitate boric acid throughout the block.

DAVID P. LAVIETES.